

## UNITED STATES PATENT OFFICE.

SUBSTITUTE FOR MISSING XR

JAMES HOWARD YOUNG, OF PITTSBURGH, PENNSYLVANIA, ASSIGNOR TO H. H. ROBERTSON COMPANY, OF PITTSBURGH, PENNSYLVANIA, A CORPORATION OF PENNSYLVANIA.

FIRE-RESISTING ASPHALT OR LIKE HYDROCARBONACEOUS MATERIAL.

1,398,991.

Specification of Letters Patent.

Patented Dec. 6, 1921.

No Drawing.

Application filed April 16, 1920. Serial No. 374,384.

To all whom it may concern:

Be it known that I, JAMES HOWARD YOUNG, a citizen of the United States, residing in Pittsburgh, in the county of Allegheny and State of Pennsylvania, have invented an Improvement in Fire-Resisting Asphalt or like Hydrocarbonaceous Material, of which the following description, in connection with the accompanying drawings, is a specification.

This invention relates to asphalt, tar, pitches, bitumens and like hydrocarbonaceous materials and has for its object to render such materials practically non-inflammable, whereby their usefulness in the industrial arts and especially in the building art may be greatly enhanced.

Strictly speaking, compounds of the hydrocarbon class are more or less inflammable, as any of them will char or burn if heated long enough and at a temperature sufficiently high, but it is possible to render asphalt, tar, pitch, bitumens and like hydrocarbonaceous materials so highly resistant to flames as to permit them to be characterized as practically non-inflammable inasmuch as they can be so modified that their rate of combustion and the heat produced is such that their kindling temperature is not spontaneously or inherently maintained and consequently combustion will proceed only when heat is supplied from an external source.

To illustrate: If a part of an area covered with the modified asphalt should be heated, only that part located in the heated zone would char, as the flame would not be carried by the modified asphalt to a part outside of the heated zone, and in this sense the term non-inflammable is herein used.

Ordinary asphalt, tar, pitch, bitumens and like hydrocarbonaceous materials in general are being used in increasing quantities for purposes where it is highly desirable that the asphalt or the like should possess non-inflammable qualities, such as in roofing products, etc. Heretofore the tendency of asphalt and the like to burn has been reduced by incorporating therewith inert non-combustible material, such as sand, chalk, slate, iron oxid, etc., and by surfacing asphalt products with such materials.

For some purposes, it is not desirable to have a large quantity of these inert mate-

rials either incorporated with or surfaced on the asphaltic product, in which case it is still desirable to reduce the fire hazard of the asphalt, which is accomplished in accordance with the present invention by incorporating with the asphalt, tar, pitch or the like when in a melted state, a material which will flux therewith, which is volatile at the relatively high temperature of 250° C. or over and gives off vapors which are non-combustible within the ordinary meaning of the term, which dilute the combustible vapors from the asphalt so that the latter is rendered inherently incapable of supporting a flame, and which will not decrease the weather-resisting or other desirable properties of the asphalt.

A suitable material for use as a modifier of the asphalt and the like is a halogen substitution product of naphthalene, and I prefer to use the chlorin substitution product on account of its relatively lower cost.

When the halogen is combined in the ring or closed chain of naphthalene, the resulting compound is very stable, will not hydrolyze at ordinary temperatures to any appreciable extent and has no detrimental action on steel.

The chlorin substitution products may be produced by subjecting melted naphthalene under pressure to the action of chlorin gas. The chlorinated products are subsequently washed with an alkali to neutralize the hydrochloric acid present, after which they are distilled.

The chloro-naphthalene products which I have found to be most effective are the solid more highly chlorinated ones.

The percentage of the chloro-naphthalene used in the asphalt or the like may vary as it depends upon the extent of chlorination of the naphthalene, the flash point of the asphalt or the like, and the degree of flame resistance which is required in the final product. About 30% of a solid chloro-naphthalene in an asphaltic composition will usually result in a product which is sufficiently flame-resisting to meet most requirements of use.

By increasing the percentage of the chloro-naphthalene in the asphaltic or like composition, the fire resistance of the latter may be increased.

The improved or modified asphaltic or

like hydrocarbonaceous material may be employed for all uses to which the untreated asphaltic or like materials are now used with the distinct advantage of reducing the fire hazard by such use, without diminishing the other advantages of the asphalt and the like, especially for building purposes.

I claim:

1. A new composition of matter consisting  
10 of bituminous material having incorporated therewith chloro-naphthalene products.
2. A new composition of matter consisting

of bituminous material having incorporated therewith chloro-naphthalene products in such quantities that the resulting composition is practically non-inflammable. 15

3. As a new article of manufacture, a bituminous material having incorporated therewith a halogen substitution product of naphthalene. 20

In testimony whereof, I have signed my name to this specification.

JAMES HOWARD YOUNG.